

W. S. ROCKEY & H. ELDRIDGE,  
PROCESS OF FUSING AND PURIFYING METALS.  
APPLICATION FILED MAY 15, 1911.

1,057,882.

Patented Apr. 1, 1913.



Witnesses:  
Samuel Hebig  
Green B. Raum

Inventors:  
Walter S. Rockey  
William Eldridge  
Frank W. Schley

# UNITED STATES PATENT OFFICE.

WALTER S. ROCKEY AND HILLIARY ELDRIDGE, OF NEW YORK, N. Y., ASSIGNEES TO  
METALLURGICAL RESEARCH COMPANY, A CORPORATION OF ARIZONA.

## PROCESS OF FUSING AND PURIFYING METALS.

1,057,882.

Specification of Letters Patent.

Patented Apr. 1, 1913.

Application filed May 15, 1911. Serial No. 627,189.

To all whom it may concern:

Be it known that we, WALTER S. ROCKEY and HILLIARY ELDRIDGE, citizens of the United States, both residing at New York, 5 in the county of New York and State of New York, have invented certain new and useful Improvements in the Process of Fusing and Purifying Metals, of which the following is a full, clear, and exact specification.

This invention relates to the fusion of metals such as copper and particularly to the fusion of electrolytic copper and to the maintenance of its purity during fusion and 15 further purification after fusion.

The object of our invention is to fuse copper and particularly cathode or electrolytic copper, and other metals to which this process may apply, by exposing it to a fuel 20 flame, or a reducing flame, in the presence of highly heated gases, products of combustion and products of gaseous and vapor decomposition which are produced by the burning of a carbonaceous, or a hydro-carbon fuel, and protecting said metal after it 25 has been fused from oxidation by an atmosphere of the gases and other products generated from the combustion of said fuel as more fully hereinafter set forth, while the 30 molten metal is flowing from the fusion chamber to the ladle, and also while the metal is flowing into said ladle and also while the metal is being poured from the ladle into casting molds.

35 A further object of our invention is to purify the copper, or metal being treated, by exposing it while in this molten condition not only to the protective but also to the reducing action of gases upon cuprous 40 compounds by the products of combustion and gaseous and vapor decomposition such as carbon monoxid, hydrogen and carbon, which may result from imperfect combustion of the fuel, or may be admitted to the 45 fusing chamber by separate means in case it is desirable to use a reducing flame secured by a perfect combustion of the fuel. We have found that when the copper is 50 acted upon by fuel which has been completely burned or if there is an excess of air or oxygen present, the gases do not act upon the copper to reduce the oxids, and it is therefore necessary to have an excess of hydro-carbon gases present to act upon and

reduce the oxids. These gases may be introduced with the fuel or the gases may be incompletely burned, thereby furnishing reducing gases necessary to purify the metal and properly effect the reduction.

In the following specification it will be 60 understood that our process may be used for fusing and purifying certain other metals other than copper, but in describing the process we will take copper as an example by which to illustrate our improvement in this art.

It has been found that electrolytic copper, which is of a high degree of purity, is contaminated by oxygen in the fusing operation where the oxygen is permitted to 70 come in contact with the copper during said operation, forming high and low oxids of copper such as  $CuO$  and  $Cu_2O$ . By our process, these impurities derived from the oxygen during fusion are eliminated by the 75 reducing action of carbon and carbon monoxid and hydrogen which are the products of combustion and gaseous and vapor decomposition, thereby providing a cheap 80 process of fusing the metal in the open flame, and thereafter protecting the molten metal by inert gases such as carbon dioxid and purifying same by the reducing action of the products of combustion, carbon monoxid or the products of decomposition, 85 hydrogen and carbon, or if perfect combustion of the fuel can be attained within the fusing chamber and no surplus of oxygen is admitted thereto during the fusing of the 90 copper, a reducing flame may be formed in which the copper is fused and the inert gases generated will protect the fused copper and prevent ingress of the outer atmosphere, so that the copper may be conducted 95 from the fusing chamber through the flue chamber, and into the ladle under the protection of said inert gases, thereby effectually preventing the oxygen of the atmosphere from coming into contact with the copper until the copper has been flowed 100 from the ladle and into the casting molds.

The process consists in locating and fusing the copper on a hearth in a fuel flame and atmosphere of incandescent and burning gases, products of combustion and products of gaseous and vapor decomposition and then flowing said copper during and after fusion as may be desired away and

from said hearth out through a downward inclined or horizontal chamber which serves both as a conduit for the flowing of the fused copper and also as a flue or chimney 5 for the outlet of flame, incandescent and burning gases, products of combustion and products of gaseous and vapor decomposition. The fused copper flowing through said conduit flue or chimney is protected 10 from atmospheric contact and consequent oxidation, by the said flame, incandescent and burning gases, products of combustion and products of gaseous and vapor decomposition, and is also purified by the reduction 15 of contained or occluded impurities by the reducing properties of said products of combustion such as carbon monoxide, and the products of gaseous and vapor decomposition such as hydrogen and carbon. This 20 protection and purification of the fused flowing copper continues by reason of the accompanying protective covering of the said flame, incandescent and burning gases, products of combustion and the products of gaseous and vapor decomposition, to the point 25 of emergence from the said conduit flue or chimney and beyond to the copper receiving ladle into which the flowing fused copper, flame, incandescent and burning gases, products 30 of combustion, products of gaseous and vapor decomposition, are discharged or precipitated together or simultaneously upon emergence from the conduit flue or chimney.

Referring to the drawings which form a 35 part of this specification, Figure 1 is a longitudinal sectional view through the furnace in which the process is carried out, and Fig. 2 is a plane view of said furnace, a portion of the hood of which is shown in 40 cross section.

In carrying out this process, we first provide a fusing furnace a modification of 45 which is shown in the annexed drawing and which is constructed of material such as silica which is refractory to heat and neutral to fused copper, and the reducing action of combustion and gaseous and vapor decomposition products. The drawing discloses a furnace which is provided with openings 50 A—A for fuel supply, a feeding orifice B, for insertion of copper, and a fusing hearth C, and a conduit flue or chimney D. A ladle E is shown for receiving the molten copper, flame and other products as previously described, and also a hood F, for carrying off the combustion products after 55 they leave the ladle. The process consists in simply heating the interior of the furnace by means of the fuel supply burners G—G, then feeding the copper through the orifice B into the furnace and on to the fusing hearth C, where it is fused, and then flowing the fused copper away from the hearth 60 and out through and out of conduit flue or chimney D and orifice H, into ladle E, the

products of combustion from thence passing off upward through the hood F, to the outer atmosphere; the orifice H may be opened by removing the plug or tap I to allow the copper to flow out of the furnace into the ladle E. The end cap J is a loose piece fitted into the end of the furnace and serves to deflect the gases, etc., downward over the flowing metal as it enters the ladle which protects the metal from the atmosphere. 70

Having thus described our invention what we claim as new is:

1. The process of fusing and purifying copper consisting in melting the copper in a fusing chamber by a hydro-carbon fuel flame carrying an excess of hydro-carbon, and then leading the fused copper from the fusing chamber together with and under the protection of the gases generated in the fusing chamber and in the presence of the products of gaseous and vapor decomposition in the fusing chamber to cause them to act on the oxids of copper to reduce the same. 80

2. The process of fusing copper consisting in melting copper in a fusing chamber by a hydro-carbon fuel flame and then leading the fused copper from the fusing chamber into a ladle together with and under the protection of gases generated in the fusing chamber by the combustion of the fuel and causing the said gases and other products to act on the said copper while and during the period that the copper is flowing through the chamber into the ladle. 85

3. The process of fusing and refining copper consisting in melting same in a fusing chamber by a fuel flame of incandescent and burning gases, and then flowing said copper during and after fusion through and out of the fusing chamber simultaneously with and beneath the protective and reducing covering of said fuel flame, incandescent and burning gases, products of combustion and products of gaseous and vapor decomposition to cause the said products to act upon the oxids and other impurities contained in the copper, thereby purifying and protecting the fused copper from contamination and oxidation to the point of emergence from the furnace. 100

4. The process of fusing copper consisting in melting copper in a fusing chamber by a hydro-carbon fuel flame, and then leading the fused copper from the fusing chamber into a ladle under the projection of gases from the fusing chamber. 105

5. The process of fusing copper consisting in melting the copper in a fusing chamber by a hydro-carbon fuel flame, and then leading the copper after fusion into a ladle beneath the protective covering of the gases and other products generated in the fusing chamber. 110

6. The process of fusing and refining copper consisting in fusing same in a fuel flame 115

of incandescent and burning gases, and then flowing said copper after fusion into a ladle beneath the protective and reducing covering of said fuel flame, incandescent and 5 burning gases, products of combustion, and products of gaseous and vapor decomposition, to cause the said gases and vapors and other products to act on the impurities contained in the copper to purify the same and 10 to prevent oxygen from coming in contact with the copper during the process.

7. The process of fusing and refining metal consisting in melting same in a fusing chamber by a fuel flame of incandescent and 15 burning gases, and then flowing said metal during and after fusion through and out of the fusing chamber into a ladle simultaneously with and beneath the protective and reducing covering of said fuel flame, incandescent and burning gases, products of combustion and products of gaseous and vapor 20 decomposition to cause the said products to act upon the oxids and other impurities contained in the metal, thereby purifying and 25 protecting the fused metal from contamination and oxidation to the point of emergence from the furnace and into the ladle.

8. The process of fusing and refining metal consisting in melting same in a fusing 30 chamber by hydro-carbon fuel flame of incandescent and burning gases, and then flowing said metal during and after fusion through and out of the fusing chamber into a ladle simultaneously with and beneath the protective and reducing covering of said 35 carbonaceous or hydro-carbon fuel flame, incandescent and burning gases, products of combustion and products of gaseous and vapor decomposition to cause the said products 40 to act upon the oxid and other impurities contained in the metal, thereby purifying and protecting the fused metal from contamination and oxidation to the point of

emergence from the furnace and into the ladle.

9. The process of treating copper, which 45 comprises continuously melting a quantity of cathode copper in a reducing atmosphere, and continuously discharging the melted product from said atmosphere.

10. The process of treating copper, which 50 consists in melting cathode copper in a reducing atmosphere, and discharging the melted copper beneath a shield formed by the reducing atmosphere.

11. The process of treating copper, which 55 consists in continuously melting cathode copper by exposing it to the highly heated gases of combustion of a fluid hydrocarbon, and preventing oxidation of the molten 60 product while being discharged by discharging the molten product together with a shield of reducing atmosphere in contact with the surface adapted to be exposed.

12. The process of treating copper, which 65 consists in continuously melting a quantity of copper in a reducing atmosphere, and continuously removing the melted product together with a shield of reducing gases 70 adapted to prevent oxidation of the metal being removed.

13. The process of treating copper, which 75 consists in melting copper by exposing it to the highly heated gases of combustion of a hydrocarbon fuel, and continuously removing the liquid product beneath a shield of reducing atmosphere in contact with the molten metal.

In testimony whereof, we affix our signatures, in presence of two witnesses.

WALTER S. ROCKEY.  
HILLIARY ELDRIDGE.

Witnesses:

G. F. QUACKINBUSH,  
HENRY J. JANSSEN.